

# UNITED STATES PATENT OFFICE.

ROGER WILLIAM WALLACE AND EUGÈNE WASSMER, OF LONDON, ENGLAND.

## PROCESS FOR THE PREPARATION OF METALLIC MAGNESIUM.

1,079,079.

Specification of Letters Patent.

Patented Nov. 18, 1913.

No Drawing.

Application filed August 18, 1913. Serial No. 785,324.

*To all whom it may concern:*

Be it known that we, ROGER WILLIAM WALLACE, residing at 2 Harcourt Buildings, Temple, London, E. C., England, and EU-  
GENE WASSMER, of 42 Manor House, Marylebone Road, London, N. W., England, have invented a new or Improved Process for the Preparation of Metallic Magnesium, of which the following is a specification.

10. Our invention consists in the preparation of metallic magnesium by treating a mixture of chlorid and sulfid of the metal in an electrolytic bath.

In one way of carrying out our invention 15 magnesium chlorid or carnallite artificial or natural is fused in a suitable vessel acting as one of the electrodes of a closed electrolytic bath with a central electrode. A calculated quantity of magnesium sulfid is then 20 added gradually to the fused salt (precaution being taken to prevent admission of atmospheric air) so as to satisfy the general meaning of the following formulae:—



or



Or the sulfid and chlorid of the magnesium may be mixed and added together to the 30 fused constituents of the electrolyte. The electric current is passed through the fused mass which at once gives off vapor of sulfur chlorid and in some cases sulfur also. These vapors are allowed to pass into a vessel 35 where the sulfur is condensed and the remaining vapors of sulfur chlorid are then allowed to pass into another vessel in which they are condensed.

The magnesium in the bath may be collected 40 in any suitable manner such for example as:—(1) Drawing off that part of the formed magnesium which is in a liquid state, or, if necessary or advantageous, (2) by introducing into the bath when tapping 45 fluorspar or any other suitable flux which will cause the magnesium to agglomerate so that it can be drawn off. In selecting a flux attention must be given to any chemical reaction which might take place between the 50 flux and the other constituents of the bath.

One of the advantages obtained from the electrolysis of these salts is that the nascent chlorin combines with the sulfid so as to form sulfur chlorid which does not attack

the containing vessel and electrode or the 55 metal formed in the process (as is the case where nascent chlorin is given off in other processes) though when the bath is almost depleted of magnesium sulfid or is maintained at too high a temperature some 60 chlorin in the free state with sulfur may be given off. Another advantage is that the reaction is carried on with a less expenditure of electric current than hitherto in the electric production of metals. We have 65 found that we get good results when working with about eight or ten volts in the bath.

The process is best carried on in a closed electrolytic vessel in which a current of nitrogen or other gas inert for the purpose is 70 maintained. The process does not require a diaphragm in the bath but this may be used if desired. The electrodes may be of any suitable material which will not be attacked by the bath, graphite for example. 75 Or one might be graphite and another iron. The temperature and current densities will vary considerably according to the size, shape, &c., of the bath and electrodes.

Having thus described our invention what 80 we claim as new and desire to secure by Letters Patent is:—

1. A process for preparing metallic magnesium which consists in electrolyzing a mixture of chlorid and sulfid of the metal in 85 an electrolytic bath.

2. A process for preparing metallic magnesium which consists in fusing magnesium chlorid and then adding gradually magnesium sulfid to the fused salt and electrolyzing 90 the bath.

3. A process for preparing metallic magnesium which consists in electrolyzing a mixture of chlorid and sulfid of the metal in an electrolytic bath and then introducing 95 into the bath a suitable flux which will cause the magnesium to agglomerate so that it can be drawn off, the said flux being inert with respect to the constituents of the bath.

In witness whereof we have signed our 100 names to this specification in the presence of two subscribing witnesses.

ROGER WILLIAM WALLACE.  
EUGÈNE WASSMER.

Witnesses:

O. J. WORTH,  
W. E. ROGERS.